

Aug. 12, 1952

D. A. NEWMAN

2,606,775

MANIFOLDING

Filed March 23, 1946

Fig. 1



Fig. 2



Fig. 3



Fig. 4



INVENTOR

Douglas A. Newman

BY

Johnson, Kline and Hensel

ATTORNEYS

## UNITED STATES PATENT OFFICE

2,606,775

## MANIFOLDING

Douglas A. Newman, Port Washington, N. Y., assignor to Columbia Ribbon and Carbon Manufacturing Company, Inc., Glen Cove, N. Y., a corporation of New York

Application March 23, 1946, Serial No. 656,558

1 Claim. (Cl. 282—28)

1

This invention relates to manifolding, particularly to the manufacture of business forms having one surface adapted to receive an inscription for record purposes, and the opposite surface having a transfer coating for producing a copy of the recorded inscription on an underlying copy sheet.

It is well known in the art to apply transfer compositions to the rear surface of record sheets, either over the entire rear surface, or on selected areas thereof in registration with form material printed on the record side of the sheet, so as to transmit only data inscribed in the areas corresponding to the transfer-coated portions to the copy sheet, such application of transfer material to selected areas of the sheet being known as "spot carbonizing."

The transfer compositions employed generally contain a coloring matter, i. e. a pigment or dye-stuff, incorporated as uniformly as possible with a wax-like material to which modifying ingredients, for example softening oils, plasticizers, solvents, hardeners such as ester gums, and the like may be added. The transfer compositions are compounded to yield a substantially solid wax-like coating, but are ordinarily applied to the surface of the paper in liquid state, by printing or analogous procedures. Thus, a transfer composition of the aforesaid type may be applied in molten condition at elevated temperatures and allowed to harden on cooling, or, the mixture may contain a volatile liquid which renders the composition fluid during application, the liquid being evaporated to obtain a solid wax-like transfer coating.

An advantageous transfer coating procedure, and compositions therefor, are disclosed in my co-pending U. S. patent applications, Serial Numbers 572,699 of January 13, 1945, and 581,631 of March 8, 1945, both now abandoned, wherein a transfer composition containing a pigment, a wax and non-volatile liquid vehicle ingredients is compounded with a volatile organic liquid, the wax being dispersed in the liquid ingredients in finely divided solid form, and the composition is applied to the paper by cold-printing methods. By reason of incorporation of the volatile liquid, relatively large amounts of pigment and dispersed wax can be incorporated in the mixture, while nevertheless maintaining sufficient fluidity without heating of the printing plates for application to the latter and thence to the paper, like an ink by ordinary printing methods. After application to the surface of the paper, the volatile liquid is evaporated and the residue is temporarily fused

2

to blend the wax, pigment and vehicle together, and upon congealing, to form a continuous transfer layer.

A serious disadvantage in carbonizing the reverse side of a record sheet for manifolding purposes, particularly in spot carbonizing, lies in the tendency of the transfer material to objectionably discolor or darken the record side of the sheet by reason of penetration of the pigmented composition into the paper, or even if the pigment is retained on the surface of the paper by penetration of the oily or wax-like components into the paper rendering the latter relatively translucent. Moreover, when ordinary paper is used, the liquid components of the transfer composition gradually bleed out of the transfer layer and are absorbed by the paper, causing a virtual drying out of the transfer material during aging whereby its transfer properties are seriously impaired.

These difficulties do not arise in the manufacture of carbon paper. The latter comprises a relatively thin tissue as a foundation which is initially flooded with the transfer composition in fluid (generally molten) condition, the excess being subsequently removed before solidification. In the interim, the paper foundation absorbs a sufficient amount of transfer composition to render any subsequent absorption during aging negligible. Since the opposite side of such a sheet is not intended or required to receive inscriptions, the penetration of the transfer composition and consequent dark color of the reverse side of the sheet is of no disadvantage. In carbonizing the rear surface of a record sheet, application of an excess of transfer composition and consequent penetration of the paper thereby must be avoided as much as possible.

The foregoing difficulties in the manufacture of carbonized record sheets restricts the choice of paper therefor, particularly for those which are to be "spot carbonized," to more expensive paper specially prepared as by coatings or filters to be resistant to penetration by transfer compositions, and to a considerable extent precludes satisfactory use of common manifolding papers which are cheaper and have a porous or absorbent character. Thus, when ordinary papers are used, the darkening effect of the transfer composition tends to render inscriptions on the front surface of the carbonized portions of the sheet difficult to read, and produces an unsightly appearance. In some cases, the transfer composition strikes through to the opposite side of the sheet, rendering the sheet unmarketable for use as a business record.

I have now discovered a method for making record sheets from paper of the quality usually employed for manifolding record sheets having a transfer coating on the rear surface, and particularly on selected areas thereof, wherein the penetrating effect of the transfer composition can be so reduced as to be unobjectionable or, if desired, can be completely eliminated despite the porous or absorbent nature of the paper employed.

Briefly stated, the process of my invention comprises, first, applying to those portions of the rear surface of a porous sheet of record paper to which transfer coating is to be applied, a coating of an organic varnish sufficient in amount and of suitable viscosity to close the pores of the paper, but insufficient to penetrate substantially below the superficial portion of the paper, drying the varnish coating, and then applying a ceraceous transfer composition in liquid form solely to the varnish-coated areas, the coating being subjected to such after-treatment as may be required to render it capable of producing copies in response to inscribing pressure applied to the record side of the sheet. When opaque papers are used, the carbonized portions of a sheet, prepared in accordance with my invention, shows substantially no darkening on the record side of the transfer-coated areas; while, if the paper is relatively translucent, the darkening effect is no greater than that produced by placing an independent darkened surface under the sheet. If it is desired to eliminate this effect in relatively translucent papers, an opacifying filler such as titanium dioxide, calcium carbonate or other white or light-colored pigments, or, if desired, light-colored pigments tinted to correspond with the color of the record sheet, can be incorporated in the varnish employed as an undercoating according to my invention. In this way any darkening due to the transfer coating can be completely eliminated, so that the carbonized portions are not readily discernible from the record side of the sheet.

In the accompanying drawings which illustrate record sheets in accordance with my invention, and a preferred process for making them:

Figure 1 is a diagrammatic view of a printing press for producing record sheets in accordance with my invention.

Fig. 2 is a rear elevation of a "spot carbonized" record sheet produced thereby.

Fig. 3 is a rear elevation of a completely carbonized record sheet in accordance with my invention.

Fig. 4 is an enlarged section of a transfer-coated portion of a record sheet produced in accordance with my invention.

Generally speaking, papers employed for record sheets in manifolding, suitable for my invention, are made of sulfite stock, of any usual degree of porosity. Such paper can be treated, in accordance with my invention, either in the form of continuous strips or as separate sheets. If desired, the paper may have suitable indicia printed on the front or record side of the sheet.

The varnish or lacquer employed as an undercoating for the transfer-coated portions of the sheets is of organic nature, and can be of the oleo-resinous or spirit type, or may be a polymerizable resin intermediate. Suitable oleo-resinous varnishes generally include, for example, bodied drying oils containing driers, together with other ingredients such as gums and minor amounts of organic solvents, such mixtures drying by polymerization on exposure to air. Suit-

able spirit varnishes are solutions or resinous or similar plastic materials, natural or synthetic, in volatile organic solvents, containing modifiers such as plasticizers, such varnishes drying by evaporation of the volatile solvent. The preferred varnish composition, employed in accordance with my invention, is ordinary lithographic varnish normally used as a vehicle for printing inks, and being essentially bodied linseed oil containing small amounts of driers such as the resinates of manganese, cobalt, or lead. A suitable spirit varnish may be composed of a 10% solution of ethyl cellulose in alcohol (e. g. denatured ethyl alcohol), or a solution of shellac in alcohol, or solutions of other varnish resins or gums which are insoluble in the oily vehicle of the transfer composition) in a volatile organic solvent. Polymeric organic compounds which form a solid resinous coating can also be used, such as polyvinyl alcohol, or urea-formaldehyde polymers.

For use in my invention, the varnish applied to the record sheet should be substantially insoluble in the transfer composition to be applied thereto, and non-fusing at temperatures employed either during application of the transfer composition, or in its subsequent treatment. Thus, the use of varnishes in which some or all of the ingredients tend to harden upon raising the temperature (below their fusion point) is particularly advantageous, as in the case of oleo-resinous varnishes, which are susceptible to accelerated polymerization at elevated temperatures. Similarly, thermo-setting resins such as urea-formaldehyde polymers are desirable for application as varnishes, or as components of varnish compositions of the spirit or oleo-resinous type.

The varnishes are applied to the areas of the rear surface of the record sheet which are to receive a transfer coating, either by coating methods, for example, if the entire surface of the sheet is to be provided with a layer of varnish, or preferably by printing in the case of sheets to be "spot-carbonized." The varnish is compounded to have sufficient viscosity and is applied in such amounts that it fills the pores of the paper but does not penetrate substantially below the surface of the paper. In general, varnishes having a viscosity of at least 8 centipoises are suitable for the purposes of the invention. When the varnish has been applied to the sheet, it is dried by heating, polymerization, evaporation of volatile solvents, or exposure to air.

Transfer compositions employed in accordance with this invention are of a ceraceous nature, containing as a coloring matter, for example, a pigment such as carbon black, Milori blue or an organic pigment; or, if the composition is to be used for hectograph reproduction, the coloring matter is a water- or spirit-soluble dyestuff such as crystal violet. In conjunction with the coloring matter, the composition contains a wax or wax-like material including natural waxes (e. g. carnauba wax, beeswax, candelilla wax, montan wax, ouricury wax, shellac wax, esparto wax) as well as synthetic waxes, or wax-like organic compounds of natural or synthetic origin, for example, fatty alcohols obtained by hydrogenization of the fatty acids contained in natural fats, As modifying ingredients, the compositions may contain plasticizers such as tricresyl phosphate, softening oils such as castor oil, mineral oil and the like, and hardening materials such as ester gums. Thus, the transfer composition may contain from 10 to 25 percent of pigment, from 20 to

35 percent of wax, and from 40 to 60 percent of liquid vehicle comprising softening oils, plasticizers and the like. A portion of the wax, for example, an amount corresponding to 5 to 15 percent of the composition can be replaced by hardening agents such as ester gum. Such compositions per se exert no substantial dissolving effect when in molten condition on organic varnishes of the type specified above.

The preferred transfer compositions employed in accordance with my invention comprises a volatile liquid such as petroleum naphtha (e. g. "Solvesso #4") as a diluent for the softening oils and plasticizers but of such nature and in such proportions that a large portion of the wax remains undissolved in the liquid ingredients, the coloring matter and the undissolved wax being incorporated in the form of finely divided dispersed solids. A suitable mixture may comprise for example, about 22 percent of wax, 17.5 percent of pigment, 41 percent of non-volatile oils and plasticizers and 19.5 percent of a volatile organic liquid. This mixture when ground together without heating yields a dispersion of solid wax and pigment in a substantially saturated solution of the wax in the liquid ingredients, having a consistency similar to printing ink.

The foregoing mixture is applied without heating, by printing methods to the varnish-coated areas on the rear surface of a manifolding record sheet and the sheet is then heated, for example, by passing it over a heated roller maintained at a temperature greater than the M. P. of the dispersed wax (e. g. in excess of 185° F.), or through a heating zone, for example, a zone in which it is subjected to infrared radiation, so as to melt the wax and cause it to blend substantially uniformly with the pigment and softening oils. The volatile liquid is simultaneously evaporated, and accordingly exerts no substantial solvent effect on the varnish layer. The resulting transfer layer is prevented by the varnish from penetrating any part of the record sheet, and the appearance of the carbonized portions of the sheet is substantially undarkened, except insofar as the transfer layer may be visible by reason of the translucency of the paper.

If the paper is relatively translucent, and it is desired to hide the transfer coating on the reverse side thereof, the varnish may contain a light colored opacifying pigment such as, for example, 10% to 40% of titanium dioxide, incorporated in lithograph varnish. While pigments of other colors may be used (such as black), a white pigment is preferable so that the printer can better gauge the amount of transfer ink being deposited on the varnished surface. When such varnish compositions are employed, the transfer coating set out above remains substantially invisible from the record surface of the manifolding sheet.

Referring to the drawings, Fig. 1 illustrates the process of my invention as applied to a continuous strip or web of manifolding paper. Thus, a strip of manifolding record paper 10 prepared, for example, from sulfite pulp, having a thickness of .0025 inch, is drawn from a roll and passed with its front surface under a printing roller 11, receiving ink from a fountain roller 12 and ductor 13, the paper being backed by a platen 14, whereby it is imprinted with form material 15 shown, for example, in Fig. 2. After printing the front surface with form matter, the paper passes over printing roller 16, fed by a ductor 17 from a fountain roller 18 with a varnish composition, for

example, lithographic varnish composed essentially of bodied linseed oil containing a drier such as a resinate of manganese, cobalt or lead. The varnish is applied by the printing roller 16 in patches or spots 19 on the rear surface of the sheet in an amount such that the varnish closes the pores of the paper but does not penetrate substantially below the superficial layer of the sheet, as illustrated in Fig. 4. Thus, the varnish 20 forms a continuous film on the surface of the paper 10 and penetrates the paper only to an insubstantial extent, indicated at 21, for example, not more than 20% of the thickness of the paper. The varnish is then dried by passing the paper through a drying zone indicated at 22, whence it passes over a printing roller 23 fed by ductor 24 from a fountain roller 25 with a transfer composition containing, for example 22% dispersed wax, 17.5% pigments, 41% oils and plasticizers, and 19.5% volatile solvents. The wax in this composition is in finely divided solid form, dispersed together with the pigment in the liquid components of the mixture. The roller 22 prints said composition without heating solely on the varnish-coated areas on the rear surface of the manifolding sheet. The paper then passes through a heating zone, indicated at 26, in which the volatile solvent is evaporated and the transfer coating is melted so as to blend the wax with the pigment and the other ingredients thereof. The strip then passes through a cooling zone indicated at 27 to solidify the transfer composition, and can then be collected in the form of a roll 28, or subjected to cutting or folding if desired.

If translucent paper is used, the lithographic varnish applied by means of roller 16 may have incorporated therewith 30 percent of its weight of titanium dioxide as an opacifier. The resulting sheets have spots 29 of transfer material 30 as shown in Fig. 2 applied on the surface of the varnish-coated portions of the paper, which are prevented by the underlying varnish coating from penetrating into the paper, regardless of its porous nature.

A portion of the wax in the transfer composition may be replaced or supplemented by incorporation of a hardener such as an ester gum. Thus, the foregoing composition may contain 15% wax, and 7% of ester gum, the remaining ingredients being the same. However, to prevent the driers in the lithographic varnish from slowly altering the hardener in the transfer composition, a small amount e. g. 1.0% of an antioxidant such as a secondary polyarylamine e. g. "Akroflex C" is advantageously added to the transfer composition. Such addition prevents serious alteration from aging of the record sheet.

If desired, the entire rear surface of the sheet can be coated with varnish 19a, and likewise the entire surface can then be carbonized as shown in Fig. 3, with transfer composition 29a.

Variations and modifications may be made within the scope of this invention and portions of the improvements may be used without others.

I claim:

A record sheet for manifolding purposes comprising a sheet of porous record paper having a front surface adapted to receive a record inscription; a printed coating of lithographic varnish including a drier on at least a portion of the rear surface of the sheet, said varnish closing the pores of the paper and being disposed substantially solely on the surface and not penetrating the paper more than superficially; and spots

of fused and solidified ceraceous transfer composition having no substantial solvent effect upon said varnish, located solely on the varnish-coated areas of said paper, said transfer composition comprising wax, softening oils, a hardener susceptible to oxidation-polymerization, and an antioxidant to prevent the drier in said lithographic varnish from promoting polymerization of said hardening ingredient.

DOUGLAS A. NEWMAN. 10

#### REFERENCES CITED

The following references are of record in the file of this patent:

1. U.S. Pat. No. 89,738, Cowan, issued Jan. 10, 1869. This patent relates to a process for the manufacture of a varnish, which is a composition of resin, oil, and drier, and which is applied to a surface, such as paper, and is then fused and solidified. The composition is stated to be substantially insoluble in solvents.

2. U.S. Pat. No. 1,463,897, Lundgren, issued Aug. 7, 1923. This patent relates to a process for the manufacture of a varnish, which is a composition of resin, oil, and drier, and which is applied to a surface, such as paper, and is then fused and solidified. The composition is stated to be substantially insoluble in solvents.

3. U.S. Pat. No. 1,929,601, Miner, issued Oct. 10, 1933. This patent relates to a process for the

manufacture of a varnish, which is a composition of resin, oil, and drier, and which is applied to a surface, such as paper, and is then fused and solidified. The composition is stated to be substantially insoluble in solvents.

4. U.S. Pat. No. 1,950,982, Gookin et al., issued Mar. 13, 1934. This patent relates to a process for the

manufacture of a varnish, which is a composition of resin, oil, and drier, and which is applied to a surface, such as paper, and is then fused and solidified. The composition is stated to be substantially insoluble in solvents.

5. U.S. Pat. No. 2,068,268, Francis, issued Feb. 28, 1937. This patent relates to a process for the

manufacture of a varnish, which is a composition of resin, oil, and drier, and which is applied to a surface, such as paper, and is then fused and solidified. The composition is stated to be substantially insoluble in solvents.

6. U.S. Pat. No. 2,301,854, Carman, issued Sept. 21, 1942. This patent relates to a process for the

manufacture of a varnish, which is a composition of resin, oil, and drier, and which is applied to a surface, such as paper, and is then fused and solidified. The composition is stated to be substantially insoluble in solvents.

7. U.S. Pat. No. 2,327,215, Potter, issued Sept. 27, 1943. This patent relates to a process for the

manufacture of a varnish, which is a composition of resin, oil, and drier, and which is applied to a surface, such as paper, and is then fused and solidified. The composition is stated to be substantially insoluble in solvents.

8. U.S. Pat. No. 2,338,176, Goepfert, issued Jan. 4, 1944. This patent relates to a process for the

#### UNITED STATES PATENTS

| Number    | Name          | Date          |
|-----------|---------------|---------------|
| 89,738    | Cowan         | May 4, 1869   |
| 1,463,897 | Lundgren      | Aug. 7, 1923  |
| 1,929,601 | Miner         | Oct. 10, 1933 |
| 1,950,982 | Gookin et al. | Mar. 13, 1934 |
| 2,068,268 | Francis       | Jan. 19, 1937 |
| 2,301,854 | Carman        | Nov. 10, 1942 |
| 2,327,215 | Potter        | Aug. 17, 1943 |
| 2,338,176 | Goepfert      | Jan. 4, 1944  |

#### FOREIGN PATENTS

| Number  | Country       | Date |
|---------|---------------|------|
| 324,859 | Great Britain | 1930 |